

1

3,651,098

### POLYGLYCIDYL ESTERS

Alfred Heer, Birsfelden, and Karl Metzger, Aesch, Basel-  
land, Switzerland, assignors to Ciba Limited, Basel,  
Switzerland

No Drawing. Filed Jan. 21, 1969, Ser. No. 792,749  
Claims priority, application Switzerland, Jan. 29, 1968,

1,314/68

Int. Cl. C07d 1/18

U.S. CL. 260—348 A

11 Claims

### ABSTRACT OF THE DISCLOSURE

Polyglycidyl esters of formula



wherein  $R_1$  and  $R_2$  independently of each other denotes a residue, obtained by removal of the carboxyl groups, or an aliphatic or cycloaliphatic polycarboxylic acid having 2 to 4 carboxyl groups, A represents the residue, obtained by removal of the two hydroxyl groups, of a polyalkylene glycol of average molecular weight of at least 200, and wherein  $m$  and  $n$  denote integers having a value of at least 1 and at most 3, preferably 1 or 2.

The subject of the present invention is new long-chain polyglycidyl esters containing aliphatic or cycloaliphatic acid residues, of general formula



wherein  $R_1$  and  $R_2$  independently of each other denote a residue, obtained by removal of the carboxyl groups, of an aliphatic or cycloaliphatic polycarboxylic acid having 2 to 4 carboxyl groups, A represents the residue, obtained by removal of the two hydroxyl groups, of a polyalkylene glycol of average molecular weight of at least 200, and wherein  $m$  and  $n$  denote integers having a value of at least 1 and at most 3, preferably 1 or 2.

Amongst the polyglycidyl esters according to the invention, of Formula I, the symmetrical compounds in which  $R_1=R_2$  and  $m=n$  can be most easily manufactured. Furthermore such polyglycidyl esters, in which  $R_1$  and  $R_2$  denote the residue of a mononuclear cycloaliphatic polycarboxylic acid or of an aliphatic polycarboxylic acid having 2 or 3 carboxyl groups and in which the residue A is derived from a polyalkylene glycol which is built up of alkylene glycol units having 2 to 6 carbon atoms are, in addition to being distinguished by easy accessibility, also distinguished by particularly valuable technical properties.

Particularly preferred compounds are the symmetrical diglycidyl esters of formula



wherein  $R'$  denotes a cyclohexylene or cyclohexenylene residue which is unsubstituted or substituted by alkyl and  $A'$  denotes the residue, obtained by removal of the two hydroxyl groups, of a polyalkylene glycol of formula



wherein "Alkylene" is an alkylene residue having 2 to 6 carbon atoms and the number  $x$  is so chosen that the

2

average molecular weight of the polyalkylene glycol is at least 200, preferably 250 to 2500.

The polyglycidyl esters according to the invention are as a rule liquid at room temperature. The compounds derived from polyalkylene glycols having higher glycol structural units such as for example polyhexanediol are mostly solid and crystalline.

The new polyglycidyl esters of Formula I can be manufactured by reacting a partial ester of formula



wherein  $R_1$ ,  $R_2$ ,  $A$ ,  $m$  and  $n$  have the same significance as



in Formula I and "Cat" denotes a cation, preferably hydrogen or alkali metal, in a single stage or several stages, with an epihalogenohydrin or  $\beta$ -methylepihalogenohydrin with elimination of "Cat-Hal," denotes the halogen atom of the epihalogenohydrin or  $\beta$ -methylepihalogenohydrin, in a manner which is in itself known. It is for example possible to proceed by reacting alkali salts of the partial esters, such as for example the di-sodium salt of the half-ester from 1 mol of a polypropylene glycol of molecular weight 425 and 2 mols of hexahydropthalic anhydride at elevated temperature with an excess of the epihalogenohydrin or  $\beta$ -methylepihalogenohydrin such as epichlorhydrin or  $\beta$ -methylepichlorhydrin, filtering off the

inorganic salt which has separated out and distilling off the excess epichlorhydrin.

It is furthermore possible to react the partial ester in the form of the free acid with an excess of epihalogenohydrin, that is to say as a rule in an amount of more than 2 mols per free carboxyl group, in the presence of suitable catalysts such as for example tertiary amines quaternary ammonium salts or ion exchanger resins, in a single stage to give the glycidyl ester. In this reaction the corresponding halogenohydrin ester first forms, with the epihalogenohydrin adding to the free carboxyl groups of the half-ester. The excess epihalogenohydrin then eliminates hydrogen halide from the halogenohydrin ester groups with the formation of glycidyl ester groups and of an equivalent quantity of glycerine dihalogenohydrin. The latter is distilled off after the completion of the reaction, together with epihalogenohydrin, and can be regenerated by treatment with strong alkalis to give the epihalogenohydrin. Such a single-stage catalytic process is for example described in German patent specification 1,165,030. The process suffers from the disadvantage of yielding relatively impure products which, as a result of major proportions of halogenohydrin esters, possess a relatively low epoxide oxygen content and a high halogen or chlorine content.

The new glycidyl esters according to the invention, of Formula I, are preferably manufactured by reacting an epihalogenohydrin, preferably epichlorhydrin, in the presence of a catalyst such as preferably a tertiary amine or a quaternary ammonium base or a quaternary ammonium salt, with a partial ester of Formula IV and treating the resulting product containing halogenohydrin groups with reagents which remove hydrogen halide.

Suitable catalysts for the addition of epichlorhydrin are above all tertiary amines such as triethylamine, tri-n-propylamine, benzylidimethylamine, N,N'-dimethylaniline and triethanolamine; quaternary ammonium bases such as benzyltrimethylammonium hydroxide; quaternary ammonium salts such as tetramethylammonium chloride, tetraethylammonium chloride, benzyltrimethylammonium chloride, benzyltrimethylammonium acetate, methyltriethylammonium chloride; and furthermore ion exchanger resins having tertiary or quaternary amino groups, and also trialkylhydrazonium salts such as trimethylhydrazonium iodide.

Suitable catalysts are furthermore also low molecular thioesters and sulphonium salts or compounds which can change into thioethers or sulphonium compounds with the epihalogenohydrins, such as hydrogen sulphide, sodium sulphide or mercaptans.

As such thioethers or sulphonium salts there may be mentioned: diethyl sulphide,  $\beta$ -hydroxyethyl ethyl sulphide,  $\beta$ -hydroxypropyl ethyl sulphide,  $\omega$ -hydroxy-tetramethylene ethyl sulphide, thioglycol, mono- $\beta$ -cyanoethyl thioglycol ether, dibenzyl sulphide, benzyl ethyl sulphide, benzyl butyl sulphide, trimethylsulphonium iodide, tris( $\beta$ -hydroxyethyl)sulphonium chloride, dibenzylmethylsulphonium bromide, 2,3-epoxypropylmethylethylsulphonium iodide, dodecyl methyl sulphide and dithiane.

Strong alkalis such as anhydrous sodium hydroxide or aqueous sodium hydroxide solution are as a rule used for the dehydrohalogenation but it is also possible to employ other alkaline reagents such as potassium hydroxide, barium hydroxide, calcium hydroxide, sodium carbonate or potassium carbonate.

The dehydrohalogenation can in turn be carried out in several stages. Thus it is possible first to treat at elevated temperature with solid sodium or potassium hydroxide and after distilling off the excess epihalogenohydrin to heat in an inert solvent with a less than equivalent amount of concentrated alkali hydroxide solution, for example 50% strength sodium hydroxide solution, as is described in German published specification 1,211,177.

Possible epihalogenohydrins are epibromhydrin and above all epichlorhydrin. Good yields are obtained if an excess of epichlorhydrin, and in particular preferably 5 to 40 mols of epichlorhydrin per carboxyl group, are used. During the first reaction, before the addition of alkali, a partial epoxidation of the bischlorhydrin ester of the partial ester (IV) already takes place. The epichlorhydrin, which acts as a hydrogen chloride acceptor is thereby partially converted to glycerine dichlorhydrin. This is again regenerated to give epichlorhydrin on treatment with alkali.

With this preferred process variant last described excellent results can be obtained especially also in the glycidylation, according to the invention, of the condensation products of 2 mols of an aliphatic or cycloaliphatic polycarboxylic acid anhydride and 1 mol of a long-chain polyalkylene glycol. The procedure developed for this new group of glycidyl esters which confer flexibility is also economically interesting since it is possible to work under very concentrated conditions (solutions of 38-50% of glycidyl compound in the epichlorhydrin) and since the yields are in general good, that is to say amount to between 93% and 99% of theory. The epoxide content of the technical products is then as a rule between 93 and 100% of theory and the chlorine content between 0 and 1.2%.

Processes for the manufacture of the polyglycidyl esters of partial esters from 1 mol of a low molecular polyalcohol or glycol (molecular weight at most about 150) such as ethylene glycol, diethylene glycol or triethylene glycol and  $n$  or 2 mols of a dicarboxylic acid anhydride such as phthalic anhydride have already been described in the patent literature (compare British patent specification 884,033 and German published specifications 1,165,030 and 1,168,907). The partial esters can either be

separately manufactured in one stage and then converted with epichlorhydrin into the polyglycidyl esters (compare German published specification 1,165,030), or the partial esters are produced on glycidylation in situ by reacting a mixture of epichlorhydrin, dicarboxylic acid anhydride and polyalcohol or polyglycol. These known processes use ion exchangers as addition catalysts, as well as using a very large excess of epichlorhydrin (the solutions contain only 3.5-6.9% by weight of ester-carboxylic acid in the epichlorhydrin) and for this reason these processes are economically less interesting because of the epichlorhydrin losses which can never be avoided. The technical crude products obtained according to the known processes show high chlorine contents (3-10%) so that they cannot be considered for many technical applications because of the corrosion properties.

The partial esters of Formula IV used as starting compounds can for example be manufactured according to known processes by reaction of 2 mols of an aliphatic or cycloaliphatic polycarboxylic acid anhydride with 1 mol of a polyalkylene glycol of formula



wherein the symbol A has the same significance as in Formula I and wherein the polyalkylene glycol (V) has an average molecular weight of at least 200, preferably 250-2500.

As suitable aliphatic polycarboxylic acid anhydrides there may be mentioned: succinic anhydride, dodecyl succinic anhydride, adipic acid polyanhydride, sebatic acid polyanhydride; 4-carboxybutane-1,2-dicarboxylic acid anhydride, maleic anhydride, adducts of maleic anhydride to unsaturated aliphatic hydrocarbons such as dipentene or tetrapropylene.

Suitable cycloaliphatic polycarboxylic acid anhydrides are for example: hexahydrophthalic anhydride, 4-methylhexahydrophthalic anhydride,  $\Delta^4$ -tetrahydrophthalic anhydride, 4-methyl- $\Delta^4$ -tetrahydrophthalic anhydride and the isomer mixtures obtained by isomerisation of tetrahydrophthalic anhydride in the presence of suitable catalysts such as metallic palladium or ruthenium (compare U.S. Pat. specification 2,764,597), which contain 4-methyl- $\Delta^3$ -tetrahydrophthalic anhydride, 4 - methyl -  $\Delta^1$  - tetrahydrophthalic anhydride and 4-methyl -  $\Delta^2$  - tetrahydrophthalic anhydride as the main components; furthermore, cyclic 1:1 adducts of maleic anhydride to compounds such as cyclopentadiene (=nadic anhydride), methylcyclopentadiene (=methyl nadic anhydride), hexachlorocyclopentadiene (=chlorendic anhydride), natural or isomerised unsaturated fatty acids such as oleic acid, linseed oil fatty acid (=Admerginate acid), anthracene,  $\beta$ -naphthol and others.

Possible polyalkylene glycols of Formula V are above all the polyethylene glycols, polypropylene glycols, polybutylene glycols or polyhexanediols having an average molecular weight of at least 200, and preferably molecular weights of about 250 to about 2500.

The new polyglycidyl esters, according to the invention, of Formula I react with the usual curing agents for epoxide compounds and can therefore be cross-linked or cured by adding such curing agents, analogously to other polyfunctional epoxide compounds or epoxide resins. Possible curing agents of this kind are basic or acid compounds.

The curing properties of the polyglycidyl esters (I) can vary depending on the acid strength of the polycarboxylic acid incorporated. Derivatives of strong dicarboxylic acids ( $p_K$ -value less than 4) as a rule already cure completely in the cold with amine curing agents whilst derivatives of weaker polycarboxylic acids as a rule can only be cured by warming.

As suitable curing agents there may for example be mentioned: amines or amides such as aliphatic, cycloaliphatic or aromatic, primary, secondary and tertiary amines, for example monoethanolamine, ethylene diamine, hexamethylene diamine, trimethylhexamethylene diamine,

diethylene triamine, triethylene tetramine, tetraethylene pentamine, N,N-dimethylpropylene diamine-1,3, N,N-diethylpropylene diamine-1,3, 2,2-bis(4'-aminocyclohexyl)propane, 3,5,5-trimethyl-3-(aminomethyl)-cyclohexylamine ("isophorone diamine"), Mannich bases such as 2,4,6-tris(dimethylaminomethyl)phenol; m-phenylene diamine, p-phenylene diamine, bis(4-aminophenyl)-methane, bis(4-aminophenyl)sulphone and m-xylylene diamine; adducts of acrylonitrile or monoepoxides such as ethylene oxide or propylene oxide, to polyalkylene polyamines such as diethylenetriamine or triethylenetetramine; adducts from polyamines such as diethylenetriamine or triethylenetetramine in excess and polyepoxides such as bisphenol-A polyglycidyl ethers; ketamines, for example from acetone or methyl ethyl ketone and bis(p-aminophenyl)methane; adducts from monophenols or polyphenols and polyamines; polyamides, especially those from aliphatic polyamines such as diethylenetriamine or triethylenetetramine and dimerised or trimerised unsaturated fatty acids, such as dimerised linseed oil fatty acid ("Versamid"); polymeric polysulphide ("Thiokol"); di-cyandiamide, and aniline-formaldehyde resins; polyhydric phenols, for example resorcinol, 2,2-bis(4-hydroxyphenyl)propane or phenol-formaldehyde resins; boron trifluoride and its complexes with organic compounds such as  $\text{BF}_3$ -ether complexes and  $\text{BF}_3$ -amine complexes, for example  $\text{BF}_3$ -monoethylamine complex; acetoacetanilide- $\text{BF}_2$  complex; phosphoric acid; triphenylphosphite; polybasic carboxylic acids and their anhydrides, for example phthalic anhydride,  $\Delta^4$ -tetrahydrophthalic anhydride, hexahydrophthalic anhydride, 4-methylhexahydrophthalic anhydride, 3,6-endomethylene- $\Delta^4$ -tetrahydrophthalic anhydride, methyl-3,6-endomethylene- $\Delta^4$ -tetrahydrophthalic anhydride (=methylnadic anhydride), 3,4,5,6,7,7-hexachlor-3,6-endomethylene- $\Delta^4$ -tetrahydrophthalic anhydride, succinic anhydride, adipic anhydride, azelaic anhydride, sebacic anhydride, maleic anhydride, dodecenylnsuccinic anhydride; pyromellitic acid dianhydride or mixtures of such anhydrides.

It is furthermore possible to employ curing accelerators in the cure, and in particular when using polyamides, polymeric polysulphides or polycarboxylic acid anhydrides as curing agents; such accelerators are for example: tertiary amines, their salts or quaternary ammonium compounds, for example 2,4,6-tris(dimethylaminomethyl)phenol, benzylidimethylamine, 2-ethyl-4-methyl-imidazole, and triamylammonium phenolate; or alkali metal alcoholes such as for example sodium hexanetriolate.

The expression "curing," as used here, relates to the conversion of the above-mentioned diepoxides into insoluble and infusible cross-linked products and in fact as a rule with simultaneous shaping to give shaped articles such as castings, pressings or laminates or to give two-dimensional articles such as coatings, lacquer films or adhesive bonds.

Corresponding to the choice of the formation component of the polyglycidyl ester (I) as well as of the type of curing agent, highly flexible or slightly flexible or rubber-elastic articles are accordingly obtained. The shaped articles in general show a low water absorption, good notched strength, high tensile strength and high elongation at break. The technical products of low chlorine content of about 0.5% are furthermore distinguished by particularly advantageous corrosion behaviour (for example when used for embedding or cementing metallic conductors).

If desired, active diluents such as for example styrene oxide, butyl glycidyl ether, isoctyl glycidyl ether, phenyl glycidyl ether, cresyl glycidyl ether and glycidyl esters of synthetic highly branched mainly tertiary aliphatic monocarboxylic acids ("Cardura E"), or cycloaliphatic monoepoxides such as 3-vinyl-2,4-dioxaspiro(5,5)-9,10-epoxyundecane can be added to the diepoxides according to the invention in order to lower the viscosity.

The diepoxides according to the invention can further-

more be used as mixtures with other curable diepoxide or polyepoxide compounds. As such there may for example be mentioned: polyglycidyl ethers or polyhydric alcohols such as 1,4-butanediol, polyethylene glycols, 5 polypropylene glycols or 2,2-bis(4'-hydroxycyclohexyl)propane; polyglycidyl ethers of polyhydric phenols such as 2,2-bis(4'-hydroxyphenyl)propane (=bisphenol A), 2,2(4'-hydroxy-3',5'-dibromophenyl)propane, bis(4-hydroxyphenyl)-sulphone, 1,1,2,2-tetrakis(4'-hydroxyphenyl)ethane or condensation products of formaldehyde with phenols manufactured in an acid medium, such as phenol novolacs or cresol novolacs; polyglycidyl esters of polycarboxylic acids such as for example phthalic acid diglycidyl ester, tetrahydrophthalic acid diglycidyl ester or hexahydrophthalic acid diglycidyl ester; triglycidyl isocyanurate, N,N'-diglycidyl-5,5-dimethylhydantoin, and aminopolyepoxides such as are obtained by dehydrohalogenation of the reaction products of epihalogenohydrin and primary or secondary amines such as aniline or 4,4'-diaminodiphenylmethane; furthermore, alicyclic compounds containing several epoxide groups, such as vinylcyclohexenediepoxide, dicyclopentadiene diepoxide, ethylene glycol-bis(3,4-epoxytetrahydrodicyclopentadien-8-yl)ether, (3',4'-epoxycyclohexylmethyl)-3,4-epoxycyclohexanecarboxylate, (3',4'-epoxy-6'-methylcyclohexylmethyl)-3,4-epoxy-6-methylcyclohexanecarboxylate, bis(cyclopentyl)-ether diepoxide or 3-(3',4'-epoxycyclohexyl)-2,4-dioxaspiro(5,5)-9,10-epoxyundecane.

Curable mixtures which are suitable for the manufacture of shaped articles including two-dimensional structures and which contain the polyepoxides according to the invention, optionally together with other diepoxide or polyepoxide compounds and furthermore curing agents for epoxide resins such as polyamines or polycarboxylic acid anhydrides are therefore also a subject of the present invention.

The polyglycidyl esters according to the invention or their mixtures with other polyepoxide compounds and/or curing agents can furthermore, in any stage before curing, be mixed with the usual modifiers such as extenders, fillers and reinforcing agents, pigments, dyestuffs, organic solvents, plasticisers, levelling agents, agents which confer thixotropy, flame-inhibiting substances or mould release agents.

The following may for example be mentioned as extenders, reinforcing agents, fillers and pigments which can be employed in the curable mixtures according to the invention: anthracite tar, bitumen, glass fibres, boron fibres, carbon fibres, cellulose, polyethylene powder, polypropylene powder, mica, asbestos, quartz powder, slate powder, aluminium trihydrate, chalk powder, gypsum, antimony trioxide, bentones, silica aerogel ("Aerosil"), lithopone, barytes, titanium dioxide, carbon black, graphite, iron oxide or metal powder such as aluminium powder or iron powder.

The following are for example suitable as organic solvents for the modification of the curable mixtures: toluene, xylene, n-propanol, butyl acetate, acetone, methyl ethyl ketone, diacetone-alcohol, ethylene glycol monomethyl ether, monoethyl ether and monobutyl ether.

Didbutyl, diocetyl and dinonyl phthalate, tricresyl phosphate, trixylenyl phosphate and also polypropylene glycols can for example be employed as plasticisers for modifying the curable mixtures.

Particularly for use in the lacquer field, the new polyglycidyl esters can furthermore be partially or completely esterified in a known manner with carboxylic acids such as especially higher unsaturated fatty acids. It is furthermore possible to add other curable synthetic resins, for example phenoplastics or aminoplastics, to such lacquer formulations.

The curable mixtures can, in the unfilled or filled state, optionally in the form of solutions or emulsions, serve as laminating resins, paints, lacquers, dipping resins, 75 pregnant resins, casting resins, pressing compositions,

sinter powders, spreading and filling compositions, floor covering compositions, embedding and insulating compositions for electrotechnology, and adhesives, as well as for the manufacture of such products.

In the examples which follow the parts denote parts by weight and the percentages denote percentages by weight.

### EXAMPLE 1

#### (a) Manufacture of the partial ester

616 g. (4 mols) of hexahydrophthalic anhydride and 850 g. (2 mols) of polypropylene glycol having an average molecular weight of 425 and 4.7 equivalents of hydroxyl groups/kg. were initially introduced into a suitable reaction vessel and warmed to 130° C. whilst stirring. A slightly exothermic reaction set in. After 60 minutes at 130° C. and a further 30 minutes at 140° C. the mixture was cooled to 90° C. and a sample was titrated to determine the acid content. The titration showed 2.75 equivalents/kg. of free acid groups (theory: 2.73 equivalent/kg.), which is equivalent to practically quantitative formation of the half-ester.

#### (b) Glycidylation of the partial ester

The half-ester was mixed with 2220 g. (24 mols) of epichlorhydrin in the same reaction vessel and the temperature was kept at 90° C. 20 g. of a 50% strength aqueous solution of tetramethylammonium chloride were added and this initiated an exothermic but easily controllable reaction. The temperature was kept at between 88 and 92° C. and the course of the reaction was monitored by means of a pH-electrode. The pH measuring device initially showed a value of between 5 and 7 which slowly increased and was about 2 pH units higher after about 20 minutes. After 20 to 25 minutes the reading on the pH measuring instrument rose abruptly in about 2 minutes by about 2 pH units, and this signified the end of the addition reaction. The pH electrode was removed and a dropping funnel containing 400 g. (5 mols) of aqueous 50% strength sodium hydroxide solution was attached. The reaction mixture was cooled to 55° C. and a further 20 g. of aqueous 50% strength solution of tetramethylammonium chloride were added. The apparatus was subjected to a vacuum and the sodium hydroxide solution was allowed to run in continuously over the course of 80 to 120 minutes at 70 to 100 mm. Hg and at an internal temperature of 52 to 58° C., with the water introduced and the water formed being azeotropically distilled off with epichlorhydrin. The epichlorhydrin was separated from the water in a water separator and continuously returned to the reaction mixture. A total of 300 ml. of water was separated off.

For working up, the apparatus was vented and the reaction mixture was successively washed in the separating funnel with 1000 ml. of water, 700 ml. of aqueous 5% strength monosodium phosphate solution and 700 ml. of water whilst warm. The epichlorhydrin solution is very concentrated (45% solids content) and can therefore in isolated cases form stable emulsions on washing. It was possible to destroy such emulsions by adding 100 to 250 ml. of ethanol. The epichlorhydrin solution was concentrated in a rotary evaporator under a water-jet vacuum. The residue was dried for 45 minutes at 120° C. under a vacuum of about 1 mm. Hg and then filtered through a pressure filter with "Hyflo" and filter paper. 1653 g. (97.8% of theory) of a pale yellow clear liquid non-crystallising product were obtained. The analytical values were:

Epoxide content: 2.3 equivalents/kg. (97.4% of theory)

Chlorine content: 0.4%

Viscosity (at 25° C.): 1500 cp. (Hoeppler viscometer)

The product mainly consisted of the following compound



### EXAMPLE 2

The partial ester from 2 mols of hexahydrophthalic anhydride and 1 mol of polypropylene glycol of average molecular weight 1025 was manufactured in an analogous manner to that described in Example 1 and the diglycidyl ester was obtained therefrom in the same manner as in Example 1. The following amounts were employed for this purpose: 1025 g. (1 mol) of polypropylene glycol of average molecular weight 1025 and having 1.95 equivalents of hydroxyl groups/kg., 308 g. (2 mols) of hexahydrophthalic anhydride, 2221 g. (24 mols) of epichlorhydrin, 200 g. (2½ mols) of aqueous sodium hydroxide solution (50% strength) and 2× 20 g. of tetramethylammonium chloride solution, 50% strength in water. 1400 g. (96.9% of theory) of light yellow, clear, liquid non-crystallising product giving the following analytical values were thereby obtained:

Epoxide content: 1.35 equivalents/kg. (97.8% of theory)

Chlorine content: 0.37%

Viscosity (at 25° C.): 820 cp. (Hoeppler viscometer)

The product mainly consists of the following compound:



### EXAMPLE 3

The partial ester was manufactured from 2 mols of hexahydrophthalic anhydride and 1 mol of poly-tetramethylene ether glycol ("polybutylene glycol") of average molecular weight 1000, in an analogous manner to that described in Example 1, and the diglycidyl ester was obtained therefrom in the same manner as in Example 1. The following quantities were used for this purpose: 1000 g. (1 mol) of poly-tetramethylene ether glycol (commercial product of Quaker Oats Co. obtainable under the registered name "Polymeg 1000"), average molecular weight 1000, 2.02 equivalents of hydroxyl groups per kg.; 308 g. (2 mols) of hexahydrophthalic anhydride, 2221 g. (24 mols) of epichlorhydrin, 200 g. (2½ mols) of aqueous sodium hydroxide solution (50% strength) and 2× 20 g. of tetramethylammonium chloride solution, 50% strength in water.

1366 g. (96.2% of theory) of pale yellow clear liquid non-crystallising product were thereby obtained, giving the following analytical values:

Epoxide content: 1.4 equivalents/kg. (99.4% of theory)

Chlorine content: <0.2%

Viscosity (at 25° C.): 1400 cp. (Hoeppler viscometer)

The product mainly consists of the following compound:





11

Oats Co. obtainable under the registered name Polymeg 1000), 356 g. (2 mols) of methyl-3,6-endomethylene- $\Delta^4$ -tetrahydrophthalic anhydride (isomer mixture), 2220 g. (24 mols) of epichlorhydrin, 200 g. (2½ mols) of aqueous sodium hydroxide solution (50% strength) and  $2 \times 20$  g. of tetramethylammonium chloride solution, 50% strength in water.

1377 g. (93.8% of theory) of light brown clear liquid non-crystallising product were thereby obtained, giving the following analytical values:

Epoxide content: 1.3 equivalents/kg. (95.4% of theory)

Chlorine content: 0.6%

Viscosity (at 25° C.): 2100 cp. (Hoeppeler viscometer)

The product mainly consists of the isomer mixture of the following compounds which are positional isomers, it being possible herein for the methyl groups to be in the 3-position, 6-position or 7-position of the bicyclic nucleus:



$n=$ about 13.6 (average value)

#### EXAMPLE 8

The partial ester was manufactured from 2 mols of 3,4,5,6,7,7-hexachlor-3,6-endomethylene- $\Delta^4$ -tetrahydrophthalic anhydride and 1 mol of polypropylene glycol of average molecular weight 425 in an analogous manner to that described in Example 1 and the diglycidyl ester was obtained therefrom in the same manner as in Example 1. The following quantities were employed: 425 g. (1 mol) of polypropylene glycol of average molecular weight 425 and having 4.70 equivalents of hydroxyl groups/kg., 742 g. (2 mols) of 3,4,5,6,7,7-hexachlor-3,6-endomethylene- $\Delta^4$ -tetrahydrophthalic anhydride, 1850 g. (20 mols) of epichlorhydrin, 200 g. (2½ mols) of aqueous sodium

35 hydroxide solution (50% strength) and  $2 \times 20$  g. of tetramethylammonium chloride solution, 50% strength in water.

1167 g. (89.2% of theory) of light brown liquid non-crystallising product were thereby obtained, giving the following analytical values:

Epoxide content: 1.25 equivalents/kg. (81.8% of theory)

Chlorine content: 2.2%

Viscosity (at 25° C.): 7500 cp. (Hoeppeler viscometer)

40 The product is not stable and at temperatures above 100° C. a volatile compound is eliminated which can be distilled off in vacuo, the epoxide content at the same time dropping slowly. The epichlorhydrin was therefore distilled off under a high vacuum and at a temperature below 95° C. The product mainly consists of the following compound:



55 hydroxide solution (50% strength) and  $2 \times 15$  g. of tetramethylammonium chloride solution, 50% strength in water.

1259 g. (98.5% of theory) of clear highly viscous liquid resin having an intense dark brown colour were thereby obtained, giving the following analytical values:

Epoxide content: 1.2 equivalents/kg. (76.7% of theory)

Chlorine content: 33.6% (101% of theory)

Viscosity (at 25° C.): 80,000 cp. (Hoeppeler viscometer)

The product mainly consists of the following compound:



$n=$ about 7 (average value)

12

#### EXAMPLE 9

The partial ester was manufactured from 2 mols of maleic anhydride and 1 mol of poly-tetramethylene ether glycol ("polybutylene glycol") of average molecular weight 1000 in an analogous manner to that described in Example 1 and the glycidyl ester was obtained therefrom in the same manner as in Example 1. The following quantities were herein employed: 1000 g. (1 mol) of polytetramethylene ether glycol of average molecular weight 1000 and having 2.02 equivalents of hydroxyl groups per kg. (commercial product of Quaker Oats Co. obtainable under the registered name Polymeg 1000), 196 g. (2 mols) of maleic anhydride, 2035 g. (22 mols) of epichlorhydrin, 200 g. (2½ mols) of aqueous sodium hydroxide solution (50% strength) and  $2 \times 20$  g. of tetramethylammonium chloride solution, 50% strength in water.

1167 g. (89.2% of theory) of light brown liquid non-crystallising product were thereby obtained, giving the following analytical values:

Epoxide content: 1.25 equivalents/kg. (81.8% of theory)

Chlorine content: 2.2%

Viscosity (at 25° C.): 7500 cp. (Hoeppeler viscometer)

40 The product is not stable and at temperatures above 100° C. a volatile compound is eliminated which can be distilled off in vacuo, the epoxide content at the same time dropping slowly. The epichlorhydrin was therefore distilled off under a high vacuum and at a temperature below 95° C. The product mainly consists of the following compound:



$n=$ about 13.6 (average value)

#### EXAMPLE 10

55 The partial ester was manufactured from 2 mols of succinic anhydride and 1 mol of polypropylene glycol of average molecular weight 1025 in an analogous manner to that described in Example 1 and the ester was glycidylated in the same manner as in Example 1. The following quantities were employed for this purpose: 1025 g. (1 mol) of polypropylene glycol of average molecular weight 1025 and having 1.95 equivalents of hydroxyl groups per kg., 200 g. (2 mols) of succinic anhydride,



1850 g. (20 mols) of epichlorhydrin, 200 g. (2½ mols) of aqueous sodium hydroxide solution (50% strength) and 2× 17 g. of tetramethyl-ammonium chloride solution, 50% strength in water.

1330 g. (99.5% of theory) of light yellow, clear, liquid non-crystallising product were thereby obtained, giving the following analytical values:

Epoxide content: 1.25 equivalents/kg. (83.6% of theory)

Chlorine content: 1.95%

Viscosity (at 25° C.): 410 cp. (Hoeppler viscometer)

The product mainly consists of the following compound:



*n*=about 17.5 (average value)

#### EXAMPLE 11

The partial ester was manufactured from 2 mols of



glutaric acid anhydride and 1 mol of polyethylene glycol of average molecular weight 1450 in an analogous manner to that described in Example 1 and this ester was glycidylated in the same manner as in Example 1. The following quantities were employed for this purpose:

1450 g. (1 mol.) of polyethylene glycol of average molecular weight 1450 (commercial product of Union Carbide obtainable under the registered name Carbowax 1540)—the material was dried for 4 hours at 140° C. under a high vacuum before use and then had 1.38 equivalents of hydroxyl groups per kg.; 228 g. (2 mols) of glutaric acid anhydride, 2775 g. (30 mols) of epichlorhydrin, 200 g. (2½ mols) of aqueous sodium hydroxide solution (50% strength) and 2× 25 g. of tetramethylammonium chloride solution, 50% strength in water.

Since the end product is partially soluble in water, the working up of the reaction mixture after completion of the addition of the sodium hydroxide was not effected as in Example 1 but as in Example 6. 1710 g. (92.5% of theory) of pale yellow clear liquid product were obtained, and this crystallised at room temperature to give a white wax-like mass. The product gave the following analytical values:

Epoxide content: 1.05 equivalents/kg. (94% of theory)  
Chlorine content: 0.6%

The product mainly consists of the following compound:



*n*=about 32.5 (average value).

#### EXAMPLE 12

The partial ester was manufactured from polysebacic acid anhydride and polyhexamethylene ether glycol (polyhexanediol) of average molecular weight 1250 in an analogous manner to that described in Example 1 and glycidylated in the same manner as in Example 1. The following quantities were employed for this purpose:

1250 g. (1 mol) of polyhexamethylene ether glycol of average molecular weight 1250 and having 1.6 equivalents of hydroxyl groups per kg., manufactured from 1,6-hexanediol in the usual manner, 388 g. of polysebacic acid

anhydride containing 0.515 equivalents of free acid groups per kg. and having a calculated anhydride group content of 5.15 equivalents/kg., 2775 g. (30 mols) of epichlorhydrin, 216 g. (2.7 mols) of aqueous sodium hydroxide solution (50% strength) and 2× 25 g. of tetramethylammonium chloride solution, 50% strength in water.

1694 g. (96.2% of theory) of pale yellow clear liquid product were obtained, which on cooling crystallised and solidified to a light grey wax-like mass. The analytical results were:

Epoxide content: 1.2 equivalents/kg. (96% of the calculated value)

Chlorine content: 0.45%

The product contains 1.5 to 2% of sebacic acid diglycidyl ester, with the remainder consisting mainly of the following compound:



*n*=about 12 (average value)

#### EXAMPLE 13

35 The partial ester was manufactured from 2 mols of 3 - alkyl - 6 - alkylene carboxy -  $\Delta^4$  - tetrahydrophthalic anhydride ("Admerginat A" of Brinckman & Mergell G.m.b.H.) and 1 mol of polypropylene glycol of average molecular weight 600, in an analogous manner to that described in Example 1, and the tetraglycidyl ester was 40 obtained therefrom in the same manner as in Example 1.



"Admerginat A," a mixture of two isomeric compounds  $C_{22}H_{34}O_5$  ( $M=378.5$ )

55 The following quantities were employed: 600 g. (1 mol) of polyethylene glycol of average molecular weight 600 (product of Union Carbide obtainable under the regis-

tered name Carbowax 600)—the material was dried for 4 hours at 140° C. under a high vacuum before use and then had 3.35 equivalents of hydroxyl groups per kg.; 870 g. of "Admerginat A" having an anhydride content of 2.3 equivalents/kg. (87% of theory) and a saponification number of 407 (91.5% of theory), 2400 g. (26 mols) of epichlorhydrin, 430 g. (5.375 mols) of aqueous sodium hydroxide solution (50% strength) and 2× 25 g. of tetramethylammonium chloride solution, 50% strength in water.

The working up of the reaction mixture after completion of the addition of the sodium hydroxide solution was not effected as in Example 1 but as in Example 6. 1690 g.

## 15

(98.7% of theory) of light clear brownish-red liquid non-crystallising product were obtained. The analytical results were:

Epoxide content: 2.2 equivalents/kg. (93.2% of theory)

Chlorine content: 0.3%

Viscosity (at 25° C.): 7900 cp. (Hoeppeler viscometer)

The product mainly consists of a mixture of isomeric compounds, for example of



$n$ =about 13.2 (average)

## 16

gether with a liquid epoxide resin C manufactured in the usual manner from bisphenol A and epichlorohydrin in the presence of sodium hydroxide and having an epoxide content of 5.3 equivalents per kg., and together with benzylidimethylamine as the accelerator, with hexahydrophthalic anhydride with gentle warming to give a homogeneous melt and were cast in siliconised 4 mm. tensile rod moulds according to DIN 53,455. The samples were cured for 12 hours at 120° C. and the tensile



strength according to DIN and the elongation at break were determined.

| Glycidyl ester according to Example No.                                       | 1         | 1     | 2     | 3     | 4     | 4     | 7     | 12    |
|-------------------------------------------------------------------------------|-----------|-------|-------|-------|-------|-------|-------|-------|
| Parts by weight of glycidyl ester                                             | 0         | 100   | 100   | 24    | 24    | 24    | 50    | 33    |
| Parts by weight of epoxide resin C                                            | 50        | ----- | 40    | 40    | 40    | ----- | 33    | 50    |
| Parts by weight of hexahydrophthalic anhydride                                | 40        | 33    | 33    | 36    | 36    | 36    | 8.5   | 33    |
| Parts by weight of benzylidimethylamine                                       | 0.2       | 0.2   | 0.2   | 0.2   | 0.2   | 0.15  | 0.2   | 0.15  |
| Parts by weight of quartz                                                     | 0         | 0     | 150   | 0     | 0     | 0     | 0     | 0     |
| Tensile strength according to DIN, kg./mm. <sup>2</sup>                       | 4         | 0.9   | 1.1   | 5.4   | 6.0   | 2.6   | 0.45  | 6.3   |
| Elongation at break, percent                                                  | 3         | 30    | 16    | 7     | 7.5   | 18.5  | 325   | 6.0   |
| Toughness: $\frac{1}{2} \times$ tensile strength $\times$ elongation at break | 6         | 13    | 9     | 19    | 22    | 24    | 74    | 21    |
| Appearance after cure                                                         | Clear (1) | (2)   | (1)   | (1)   | (2)   | (3)   | (1)   | (2)   |
| Water absorption in percent, 4 days at room temperature                       | 0.28      | 0.7   | ----- | 0.4   | ----- | ----- | ----- | ----- |
| Water absorption in percent, 1 hour at 100° C                                 | 0.3       | 1.7   | ----- | ----- | ----- | ----- | ----- | ----- |

<sup>1</sup> Clear yellow. <sup>2</sup> Opaque grey. <sup>3</sup> Opaque white.

## EXAMPLE 14

Some of the polyglycidyl esters manufactured according to Examples 1-13 were mixed together with a liquid cycloaliphatic epoxide resin A which had an epoxide content of 6.2 equivalents/kg., and an accelerator B which consisted of an approximately 0.8% strength solution of sodium metal in hexanetriol, as with hexahydrophthalic acid anhydride with gentle warming to give a homogeneous melt, and were cast in siliconised 4 mm. tensile rod moulds according to DIN 53,455. The samples were cured for 12 hours at 120° and the tensile strength according to DIN and the elongation at break were then determined. For comparison purposes, the product of  $\frac{1}{2} \times$  elongation at break  $\times$  tensile strength was calculated as a measure of the "toughness."



Epoxide Resin A

| Glycidyl ester according to Example No.                                        | 2     | 4         |
|--------------------------------------------------------------------------------|-------|-----------|
| Parts by weight of glycidyl ester                                              | 0     | 10        |
| Parts by weight of epoxide resin A                                             | 25    | 25        |
| Parts by weight of hexahydrophthalic anhydride                                 | 21    | 25        |
| Parts by weight of accelerator B                                               | 2.5   | 2.5       |
| Tensile strength according to DIN, kg./mm. <sup>2</sup>                        | 4.0   | 6.0       |
| Elongation at break, percent                                                   | 2.5   | 4         |
| "Toughness" $\frac{1}{2} \times$ tensile strength $\times$ elongation at break | 5     | 12        |
| Appearance after cure                                                          | Clear | Clear (1) |

<sup>1</sup> Opaque white.

## EXAMPLE 15

Some of the polyglycidyl esters manufactured according to Examples 1-13 were mixed, by themselves or to-

| Glycidyl ester according to Example No.                                       | 1    | 1    | 2    | 3    | 4    | 4    | 7    | 12   |
|-------------------------------------------------------------------------------|------|------|------|------|------|------|------|------|
| Parts by weight of glycidyl ester                                             | 90   | 90   | 90   | 90   | 90   | 90   | 90   | 90   |
| Parts by weight of epoxide resin C                                            | 10   | 10   | 10   | 10   | 10   | 10   | 10   | 10   |
| Parts by weight of hexahydrophthalic anhydride                                | 34   | 34   | 34   | 34   | 34   | 34   | 34   | 34   |
| Parts by weight of benzylidimethylamine                                       | 0.25 | 0.25 | 0.25 | 0.25 | 0.25 | 0.25 | 0.25 | 0.25 |
| Parts by weight of quartz powder                                              | 200  | 200  | 200  | 200  | 200  | 200  | 200  | 200  |
| Measured values at (° C.)                                                     | 25   | 25   | 25   | 25   | 25   | 25   | 25   | 25   |
| Tensile strength according to DIN, kg./mm. <sup>2</sup>                       | 1.2  | 2.5  | 6.6  | 28   | 20   | 8    | 28   | 20   |
| Elongation at break, percent                                                  | 28   | 20   | 20   | 20   | 20   | 20   | 20   | 20   |
| Toughness: $\frac{1}{2} \times$ tensile strength $\times$ elongation at break | 17   | 25   | 28   | 28   | 20   | 8    | 28   | 20   |

## EXAMPLE 16

| Glycidyl ester according to Example No.                                       | 2   | 3   |
|-------------------------------------------------------------------------------|-----|-----|
| Parts by weight of glycidyl ester                                             | 0   | 31  |
| Parts by weight of epoxide resin C                                            | 100 | 62  |
| Parts by weight of triethylene tetramine                                      | 10  | 7   |
| Tensile strength according to DIN, kg./mm. <sup>2</sup>                       | 4.8 | 3.5 |
| Elongation at break, percent                                                  | 2.7 | 5.2 |
| Toughness: $\frac{1}{2} \times$ tensile strength $\times$ elongation at break | 5.7 | 9   |

## EXAMPLE 17

Epoxide resin D: by way of comparison, the partial ester was manufactured from 2 mols of hexahydrophthalic anhydride and 1 mol of ethylene glycol in an analogous

manner to Example 1, and the diglycidyl ester (epoxide resin D) obtained therefrom in the same manner as in



Example 1. The yield was 91% of theory; the product had the following analytical values:

Epoxide content: 4.0 equivalents/kg. (96% of theory)  
Total chlorine content: 1.0% (according to Wurzschnitt)  
Viscosity: (at 25° C.) 9700 cp. (Hoeppler viscometer)

Epoxide resin E: the partial ester was manufactured from 2 mols of  $\Delta^4$ -tetrahydrophthalic anhydride and 1 15



mol of ethylene glycol in an analogous manner to that described in Example 1 and the diglycidyl ester (epoxide resin E) was obtained therefrom in the same manner as in Example 1. The yield was 94% of theory; the product had the following analytical values:

Epoxide content: 4.1 equivalents/kg. (98% of theory)

Total chlorine content: 1.0% (according to Wurzschmitt)

Viscosity (at 25° C.): 15000 cp. (Hoepppler viscometer)



The epoxide resins D and E manufactured according to Example 17 were cast and cured in accordance with Example 15.



| Glycidyl ester according to Example 17                                        | D    | D   | E   | E   | D   |
|-------------------------------------------------------------------------------|------|-----|-----|-----|-----|
| Parts by weight of glycidyl ester                                             | 100  | 50  | 100 | 50  | 50  |
| Parts by weight of epoxide resin C                                            |      | 50  | —   | 50  | 50  |
| Parts by weight of hexahydrophthalic anhydride                                | 61.5 | 71  | 63  | 72  | 71  |
| Parts by weight of benzylidinemethylamine                                     | 0.2  | 0.2 | 0.2 | 0.2 | 0.2 |
| Parts by weight of quartz powder                                              |      |     |     |     | 150 |
| Tensile strength according to DIN, kg./mm. <sup>2</sup>                       | 4.2  | 6.0 | 5.0 | 6.5 | 6.0 |
| Elongation at break, percent                                                  | 4    | 3   | 3.5 | 3   | 2   |
| Toughness: $\frac{1}{2} \times$ tensile strength $\times$ elongation at break | 8.4  | 9   | 8.8 | 9.8 | 6.0 |
| Water absorption in percent, 4 days at room temperature                       | 0.4  | —   | 0.4 | —   | 0.2 |



wherein "Alkylene" is an alkylene residue having 2 to 6 carbon atoms and the number  $x$  is so chosen that the average molecular weight of the polyalkylene glycol is 250 to 2500.



The polyglycidyl esters according to the invention show



a higher elongation at break and greater toughness than the diglycidyl esters manufactured in Example 17.

## 6. Diglycidyl ester of formula



## 7. Diglycidyl ester of formula



### 8. Diglycidyl ester of formula



*n=4-15*

### 9. Diglycidyl ester of formula



where  $z=2$  to 8 and  $n=4$ –35.

## 10. Diglycidyl ester of formula



wherein  $z=2$  to  $8$  and  $n=13$ – $33$ .

## 11. Diglycidyl ester of formula



wherein  $z=3$  to 8 and  $n=6$  to 20.

## References Cited

## FOREIGN PATENTS

559,078 6/1958 Canada.

**NORMA S. MILESTONE, Primary Examiner**

U.S. Cl. X.R.

260—2 EC, 2 EA, 2 N; 260—468 B, 468 R, 485 G

UNITED STATES PATENT OFFICE  
CERTIFICATE OF CORRECTIONPatent No. 3,651,098Dated March 21, 1972Inventor(s) ALFRED HEER ET AL

It is certified that error appears in the above-identified patent  
and that said Letters Patent are hereby corrected as shown below:

Column 1, line 4, after "assignors to" delete "Ciba Limited"  
and insert -- CIBA-GEIGY AG --.

Column 18, the extreme right side of the formula following

line 30,  $-\text{CH}-\text{CH}_2-$  should read  $-\text{CH}-\text{CH}_2-$

Column 19, the bottom of the formula of claim 8

$-\left[\text{CH}-\text{CH}_2-\text{O}\right]_n-$  should read  $-\left[\begin{array}{c} \text{CH}-\text{CH}_2-\text{O} \\ | \\ \text{CH}_3 \end{array}\right]_n-$

delete "n=4-15" and insert -- n=4-35 --;

the center of the formula of claim 9

$-\left[\begin{array}{c} \text{CH}-\text{CH}_2-\text{O} \\ | \\ \text{CH}_2 \end{array}\right]_n-$  should read  $-\left[\begin{array}{c} \text{CH}-\text{CH}_2-\text{O} \\ | \\ \text{CH}_3 \end{array}\right]_n-$

Signed and sealed this 25th day of June 1974.

(SEAL)  
Attest:

EDWARD M. FLETCHER, JR.  
Attesting Officer

C. MARSHALL DANN  
Commissioner of Patents